

## UNITED STATES PATENT OFFICE.

HARRY L. GRANT AND WILLIAM R. FARREN, OF TAMAQUA, PENNSYLVANIA, ASSIGNEES TO ATLAS POWDER COMPANY, OF WILMINGTON, DELAWARE, A CORPORATION OF DELAWARE.

## SEALING AND INSULATING COMPOSITION.

No Drawing.

Application filed June 25, 1925. Serial No. 39,594.

Our invention relates to compositions comprising cumarone resins and sulphur or sulphur compounds such as thio-carbanilid, thio-urea, etc., and has for its object to provide a new and more suitable dielectric material for sealing the casings and other protective containers for delicate electrical and mechanical units and containers for hygroscopic materials. A further object of this invention is to provide a highly water-proof and dielectric material which will melt and flow freely at temperatures somewhat higher than the boiling point of water enabling it to be moulded or cast in any geometric form without the aid of pressures in excess of the atmospheric pressure. Among the objects of this invention is to provide a material characterized by ease of compounding and low cost of raw materials.

In carrying out our invention use is made of the cumar or cumarone sulphur mixture for making various shaped articles, wherein a combination of water-proof and dielectric properties is desired. The articles to be produced from this material are usually made by pouring the composition, while in a molten state, into suitable moulds or cavities, thus producing moulded or cast parts. In using the material for sealing casings or protective coverings or containers it is brought to a molten state by heating and when completely molten is poured into the cavity to be sealed. Sulphur is largely used as a sealing material in many of the arts. However sulphur alone, if cast into a shape, crystallizes as it solidifies, forming a more or less porous and fragile structure. The addition of finely divided, solid materials, such as sand, clay, glass, brick dust, etc., results in the production of a less porous mass than is produced by the use of sulphur alone. The finely divided material seems to interfere with the formation of sulphur crystals, or at least, causes the formation of smaller crystals than would otherwise form. By the addition of cumar or cumarone resin to the sulphur, crystallization of the mass is completely prevented and a hard, amorphous casting is produced. We contemplate the continued use of finely divided filling materials, when desired, along with the cumar resin, though the omission of these is within the scope of the invention. A particular use has been made of our improved material for

sealing electric blasting cap shells after insertion of the so-called electric fuse head or igniting device. Exhaustive experiments have shown that electric blasting caps sealed with this material are, practically speaking, impervious to moisture. The usual material for filling such caps generally consists of sulphur, mixed with a small percentage of brick dust, graphite, powdered sand or powdered glass, etc. The electric blasting caps sealed with such compositions, however, unless special means has been employed, will not prevent the entrance of atmospheric moisture nor will they withstand water pressures much above the atmospheric pressure. Now electric blasting caps sealed with the composition of our invention have withstood water pressures as high as 70 lbs. per sq. in., i. e., above atmospheric pressure, or, roughly, 85 lbs. absolute pressure, for periods of several hours. Results of our experiments have shown that the charges in the electric blasting caps sealed with the cumar-sulphur mixture are not affected by atmospheric moisture, when protected as described. This is a very desirable property for it is well known that even traces of moisture in the charge will greatly reduce the strength of the detonator. The material described above is chemically neutral and inert toward the metal of the shell; the explosive used for charging, and also the fuse head. For special purposes we may employ compositions comprising sulphur and coal tar resins comparable with the above described cumarone resin.

The sealing elements made by our improved method may be made by casting the compositions in place or by mixing the ingredients in a dry state and fusing them by the application of heat alone, or heat and pressure.

Our improved composition may be used to advantage as a binder in a manner analogous to the use of shellac in chill molding objects, i. e. taking the composition comprising finely divided sulphur-cumar resin and inert filling material, putting it in a hot mold, pressing it to shape, chilling the mold below the solidifying point of the cumar resin and removing the shaped article from the mold.

It is to be understood that our invention is not limited to the precise compositions or

manner of use set forth in the description, but that it includes within its scope whatever changes or variations fairly come within either the spirit of the invention or the terms of the appended claims.

Having described our invention, what we claim as new and desire to secure by Letters Patent is:—

1. The herein described process of making 10 a dielectric and water-proof sealing material which consists of incorporating, into a homogeneous plastic mass only molten sulphur, molten cumarone resin and a finely divided filling material all in such proportions as to 15 produce a body that is solid when cold.

2. A water-proof and dielectric sealing 20 material of the character described consisting of a body of sulphur and cumarone resin combined in such proportions that the whole may be rendered plastic by the application

of heat and moulded or poured while in that condition, the body becoming hard when cold, and the cumarone resin preventing crystallization of the sulphur upon cooling of the mass.

3. A water-proof and dielectric sealing material of the character described consisting wholly of a body of sulphur, a finely divided filling material, and cumarone resin combined in such proportions that the whole 30 may be rendered plastic by the application of heat and moulded or poured while in that condition, the body becoming hard when cold, and the cumarone resin preventing crystallization of the sulphur upon cooling 35 of the mass.

In testimony whereof they affix their signatures.

HARRY L. GRANT.  
WILLIAM R. FARREN.